

## 1

3,544,393

**METHOD OF MANUFACTURING LOW CARBON HIGH TENSILE STRENGTH ALLOY STEEL**  
 Joseph R. Zanetti, Dearborn, Mich., assignor to National Steel Corporation, a corporation of Delaware  
 No Drawing. Filed Aug. 11, 1967, Ser. No. 659,885  
 Int. Cl. C21d 7/00

U.S. Cl. 148—12

2 Claims

**ABSTRACT OF THE DISCLOSURE**

A low carbon, weldable, high tensile strength alloy steel characterized by ductility and toughness suitable for structural uses is produced in the "as rolled" condition by utilizing a steel consisting essentially, by weight, of

|           | Percent, about |
|-----------|----------------|
| Carbon    | .10-20         |
| Manganese | .75-1.15       |
| Silicon   | .50-1.0        |
| Chromium  | .50-80         |
| Zirconium | .05-20         |
| Boron     | .0005-0.025    |
| Titanium  | .02-15         |
| Columbium | .01-06         |

and the balance iron with residual impurities. The steel is hot rolled to form bars, plate and sheets with a starting rolling temperature between 2100° F.-2300° F. and a finishing rolling temperature between 1400° F.-1700° F. followed by air cooling.

This invention is concerned with low carbon, high tensile strength, alloy steel. More specifically it is concerned with low carbon, high tensile strength, alloy steel having a minimum tensile strength of about 75,000 p.s.i. in the "as rolled" condition.

Low carbon, high tensile strength steels of the prior art have required heating, quenching, and tempering treatment subsequent to rolling in order to develop the desired tensile strengths and suitable ductility and toughness. Such treatments require multiple and uneconomical handlings, e.g., the product must be held rigidly to prevent warping while being cooled rapidly from a temperature about 1750° F., and higher, to room temperature in about 10 to 25 seconds.

The quenching develops 100% marstenitic steel and is required to obtain desired high tensile strength. Without such quench treatment, such steels have a tensile strength of about 50,000 to 60,000 p.s.i. in the "as rolled" condition.

After quenching, such steels previously required a tempering treatment at about 850° F. to about 1300° F. to develop ductility and other properties necessary for end product usage.

This invention provides an alloy steel with high tensile strengths in the range of about 80,000 to about 120,000 p.s.i. (minimum tensile strength of 75,000 p.s.i.). In addition, the steel exhibits ductility and yield point elon-

## 2

gation values suitable for normal fabrication of high tensile strength steels and toughness suitable to withstanding normal stresses encountered in use of such steels. Obtaining these results without treatment subsequent to rolling is one of the highly unexpected contributions of the invention.

The low carbon high tensile strength alloy steel of the present invention consists essentially of the following weight-percentages:

|           | Percent, about |
|-----------|----------------|
| Carbon    | .07-20         |
| Manganese | .75-1.15       |
| Silicon   | .50-1.0        |
| Chromium  | .50-80         |
| Zirconium | .05-20         |
| Boron     | .0005-.0025    |
| Titanium  | .15 max.       |
| Columbium | .01-06         |

20 the balance being iron with residual impurities such as are ordinarily encountered in conventional basic oxygen, open hearth, or electric furnace practice used in producing the steel. The maximum desirable values of the most common residual impurities encountered are:

|            |          |
|------------|----------|
| Phosphorus | .04 max. |
| Sulphur    | .05 max. |
| Copper     | .35 max. |
| Aluminum   | .07 max. |

The upper limit of carbon is ordinarily not exceeded in order to maintain the good weldability of end product provided by the invention. Carbon content below the lower limit is ordinarily avoided in order to have sufficient carbon available for providing desired tensile strength.

The manganese is added in the furnace or the ladle. Where possible, e.g., in open hearth practice, it is added in both the furnace and the ladle. Preferably, the manganese is maintained in the range of .85% to 1.0% with a specific value of .90% being desired. The manganese helps increase the yield point and tensile strength of the steel and aids cold formability.

Silicon acts as a deoxidizer and ferrite strengthener. It can be added in the furnace or ladle; where possible silicon is added in both. Silicon is desirably kept in the range of .75% to 90% with .85% being preferred.

The chromium is added in the ladle and acts to increase both the yield point and tensile strength of the steel. A preferred specific value for the chromium is .65%.

The zirconium acts to increase hardenability, refine grain structure, increase toughness and cold formability. It is added in the ladle and is preferably kept between .075% and .12%; with .08% being the specific value aimed for.

The boron is added in the ladle. It increases hardenability of the steel and seeks out remnants of nitrogen in the steel to a greater extent than other nitride formers such as chromium, zirconium, columbium. The titanium helps to protect the boron for this purpose because of its

greater affinity for oxygen than boron. A preferred value for the boron is .0010% and a preferred range is .0005% to .012%.

The titanium also acts as a carbide former and is preferably kept at about .03%. The titanium should be added with the boron.

Columbium contributes to a number of the unexpected

these properties are set forth in the representative examples below:

#### EXAMPLE No. 1

Low carbon columbium treated alloy steel bars having a minimum yield strength of 75,000 p.s.i. Dimensions: 5 1/8" x .250 x 100"; 4 1/2" x .312 x 110".

|                    | C   | Mn  | P    | S    | Si  | Cr  | Zr  | B     | Ti  | Cb   |
|--------------------|-----|-----|------|------|-----|-----|-----|-------|-----|------|
| Ladle chemistry    | .17 | .94 | .013 | .010 | .90 | .74 | .08 | .0012 | .03 | .038 |
| Recheck chemistry: |     |     |      |      |     |     |     |       |     |      |
| .250 ga.           | .17 | .94 |      |      | .87 | .75 | .09 | .0014 | .03 | .035 |
| .312 ga.           | .17 | .97 |      |      | .88 | .76 | .10 | .0014 | .03 | .037 |

#### MECHANICAL PROPERTIES

| Bars        | YS (p.s.i.) | TS (p.s.i.) | Elong. percent, in. | Bend |
|-------------|-------------|-------------|---------------------|------|
| "As rolled" |             |             | 2-4-8               |      |
| .250 ga.    |             |             |                     |      |
| Front       | 88,550      | 110,620     | 29-21-15 SB 2       | 16Xt |
| Middle      | 78,100      | 106,930     | 29-21-16 SB         | 22Xt |
| Back        | 80,540      | 111,360     | 24-16-11 SB         | 22Xt |
| .312 ga.    |             |             |                     |      |
| Front       |             | 103,760     |                     |      |
| Middle      | 81,690      | 107,180     | 28-17-14 SB         |      |
| Back        | 79,190      | 105,140     | 30-22-16 SB         |      |

<sup>1</sup> 0.2% offset. <sup>2</sup> Short break.

#### CHARPY "V" IMPACT TEST DATA

[Ft.-lb., at temperature °F.]

| Thickness              | Direction    | Rm. temp. | 32   | 0    | -20  | -40 | -60 |
|------------------------|--------------|-----------|------|------|------|-----|-----|
| .250"                  | Transverse   | 12.7      | 9.0  | 6.7  | 4.8  | 3.0 | 2.2 |
| .394" x .107" x 2.165" | Longitudinal | 24.3      | 17.7 | 13.8 | 13.8 | 6.0 | 4.2 |
| .312"                  | Transverse   | 18.7      | 10.7 | 6.5  | 4.5  | 2.8 | 2.7 |
| .394" x .295" x 2.165" | Longitudinal | 39.0      | 18.0 | 12.3 | 6.0  | 3.8 | 3.2 |

#### EXAMPLE NO. 2

|                    | C   | Mn  | P    | S    | Si  | Cu  | Cr  | Zr  | Al   | B     | Ti  | Cb   |
|--------------------|-----|-----|------|------|-----|-----|-----|-----|------|-------|-----|------|
| Ladle chemistry    | .17 | .92 | .010 | .024 | .78 | .03 | .70 | .06 | .041 | .0007 | .03 | (1)  |
| Recheck chemistry: |     |     |      |      |     |     |     |     |      |       |     |      |
| .250 ga.           | .18 | .90 | .009 | .025 | .79 | .04 | .70 | .08 | .041 | .0007 | .03 | .056 |
| .3125 ga.          | .17 | .87 | .009 | .025 | .78 | .04 | .68 | .07 | .040 | .0007 | .03 | .055 |

<sup>1</sup> Added in mold.

#### MECHANICAL PROPERTIES

| Bars        | Brinell Hardness No. | YS (p.s.i.) | TS (p.s.i.) | Elong. in. | TS/YP | Bend    |
|-------------|----------------------|-------------|-------------|------------|-------|---------|
| "As rolled" |                      |             |             | 2-8        |       |         |
| .250 ga.    | 223/241              | 81,600      | 119,730     | 14-21      | 1.37  | 1Xt     |
|             |                      | 84,600      | 119,310     | 19         | 1.41  |         |
|             |                      | 99,040      | 117,520     | 15         | 1.18  |         |
| .3125 ga.   | 212/229              | 76,200      | 102,080     | 23-33      | 1.34  | 1 1/2Xt |
|             |                      | 86,980      | 103,820     | 19         | 1.19  |         |
|             |                      | 94,280      | 103,120     | 20         | 1.09  |         |

<sup>1</sup> 0.2% offset.

#### CHARPY "V" IMPACT TEST DATA

[Ft.-lb. at temperature °F.]

| Thickness                | R/T       | 32       | 0       | -20     | -40     |       |
|--------------------------|-----------|----------|---------|---------|---------|-------|
| .250" (.394X.197X2.165)  | 7.0/4.7   | 5.5/3.3  | 4.7/3.0 | 3.2/2.5 | 2.3/2.0 | (1/t) |
| .3125" (.394X.295X2.165) | 28.0/12.3 | 15.0/7.6 | 8.8/5.8 | 4.5/3.5 | 4.5/3.0 |       |

results obtained through the invention. It raises the yield point significantly without detrimental effect on the highly desirable ductility and toughness obtained by the invention in the "as rolled" condition. The columbium is added in the ladle, or can be added in the mold. A preferred specific value for the columbium is .035% and the preferred range is .035% to .06%.

If the steel is degassed during processing the ladle additions are made after degassing to minimize oxidation products and reduce possible contamination of the steel.

The alloy steel of this invention is rolled into bars, plate or sheets which are suitable for structural uses, railway car framing, and the like. This steel is characterized by high tensile strength, good weldability, high energy absorption capacity, and good ductility and yield point elongation values in the "as rolled" condition. Data on

The process taught by the present invention, in addition to or in combination with the chemistry, also contributes to the desirable characteristics obtained. In practice the alloy steel is provided in billet form, that is in a suitable form for rolling into bars, plates or sheets. The billets are heat soaked at about 2100 to 2300° F., preferably about 2150° F., prior to rolling. The billets are then rolled. Multiple stand rolling is carried out so that finishing rolling temperature of the product of the present invention can be about 200° to 300° lower than the finishing rolling temperatures employed with high tensile strength steels in the prior art. The finishing rolling temperature should be in the range of 1400° to about 1700° F.

After rolling the product is allowed to cool without quenching or forced cooling. Such cooling will ordinarily

take place at a rate of about 5 to 10° per second at least through the major portion of the cooling depending on the shape and thickness of the final product.

Other advantages of the invention are inherent in the above description. It is understood that changes and modifications in the foregoing teachings can be made without departing from the spirit of the invention so that the scope of the invention is to be determined from the appended claims.

What is claimed is:

1. Process for producing low carbon high tensile strength alloy steel bar and plate suitable for welding and characterized by minimum tensile strength of 75,000 p.s.i. in the "as rolled" condition without subsequent heat treatment comprising the steps of

providing an alloy steel billet consisting essentially, by weight, of

Percent, about

|           |             |
|-----------|-------------|
| Carbon    | 0.7-20      |
| Manganese | .75-1.15    |
| Silicon   | .50-1.0     |
| Chromium  | .50-.80     |
| Zirconium | .05-.20     |
| Boron     | .0005-.0025 |
| Titanium  | .15 max.    |
| Columbium | .01-.06     |

and the balance iron with residual impurities,

heat soaking such alloy steel billet at a temperature between about 2100° F. and about 2300° F., hot rolling the steel billet to desired dimensions, with a hot rolling starting temperature being between about 2100° F. and about 2300° F. and a hot rolling finishing temperature between about 1400° F. and about 1700° F., and allowing the hot rolled steel to cool without quenching or forced cooling.

2. The process of claim 1 in which the hot rolling starting temperature is about 2150° F. and the hot rolled steel air cools at a rate of about 5°-10° per second.

#### References Cited

##### UNITED STATES PATENTS

|           |         |             |       |        |
|-----------|---------|-------------|-------|--------|
| 3,010,822 | 11/1961 | Altenberger | ----- | 148-12 |
| 3,102,831 | 9/1963  | Tisdale     | ----- | 148-12 |

##### OTHER REFERENCES

20 "Making, Shaping and Treating of Steel," by U.S. Steel, 7th edition, pp. 386-387.

HYLAND BIZOT, Primary Examiner

U.S. Cl. X.R.

75-126

UNITED STATES PATENT OFFICE  
CERTIFICATE OF CORRECTION

Patent No. 3,544,393 Dated December 1, 1970

Inventor(s) Joseph R. Zanetti

It is certified that error appears in the above-identified patent and that said Letters Patent are hereby corrected as shown below:



Column 2, line 39, "furance" should read --  
furnace -- (p. 4, line 3)

Column 2, line 47, "90%" should read -- .90% --  
(page 4, line 11)

Column 2, line 57, "remants" should read -- remnants  
(page 4, line 20)

Column 5, line 18, carbon percent should read --  
.07 - .20% -- (claim 4, line 8).

Signed and sealed this 28th day of September 1971.

(SEAL)

Attest:

EDWARD M. FLETCHER, JR.  
Attesting Officer

ROBERT GOTTSCHALK  
Acting Commissioner of Patents